

1

3,167,504  
**METHOD FOR PURIFYING RADIOACTIVE  
WASTE LIQUID**

Walter L. Hayden, Jr., Metuchen, and Frank J. Dzier-  
zanowski, Somerset, N.J., assignors to Minerals &  
Chemicals Philipp Corporation, Menlo Park, N.J., a  
corporation of Maryland

No Drawing. Filed Oct. 4, 1961, Ser. No. 142,764  
7 Claims. (Cl. 210—24)

This invention relates to a method for eliminating radioactive isotopic material from radioactive waste liquids and relates especially to the elimination of radio cesium from such liquids by adsorption.

The handling and disposal of radioactive wastes is a constant problem in nuclear energy operations. As the utilization of nuclear energy increases, the safe and economical disposal of radioactive waste becomes more pressing.

Most radioactive waste material is in liquid form and it is obtained, for example, by dissolving spent fuel in nitric acid. Many of the fission products present in the waste liquid have a short half-life and, therefore, their safe disposal presents no problem. The difficulty comes about as a presence in the waste liquid of radio cesium ( $Cs^{137}$ ) and radio strontium.

Radioisotopic elements in radioactive wastes are ultimately safely disposed of by burial in the ground, ocean or other geological formations of the suitable composition. The concentration of radioisotopic elements in liquid waste, especially low level waste, is too low to permit the economic disposal of the entire liquid by direct burial. Therefore, the liquid waste must undergo preliminary treatment so as to concentrate the radioactive values in the liquid. Various methods have been suggested to effect this result, as examples of which may be mentioned: evaporation of the liquid; fixation of radioisotopic elements by solids; precipitation of radioisotopic elements from the waste liquid; and calcination of the waste liquid. Some of these pretreatments of radioactive waste liquids, especially low level liquid wastes, are not economically feasible when carried out on large scale. Thus, for example, concentration of wastes by evaporation is not practical for handling large volumes of low level wastes.

One of the most practical approaches to the disposal of liquid radioactive waste liquids is the fixation of radioactive elements in the liquid waste on a solid, as by adsorption or ion-exchange, so that the liquid can be safely released to normal environmental liquid waste disposal sites or waters.

To accomplish this result it has been suggested to contact the waste liquid with certain naturally occurring minerals which are capable of selectively adsorbing radioactive elements. Montmorillonite, illite, clinoptilolite and erionite have been recommended for fixing radio cesium. All of these minerals are crystalline silicates. Montmorillonite and illite are clay minerals; clinoptilolite and erionite, which are most promising, are naturally occurring zeolites.

However, naturally occurring minerals generally have definite limitations as adsorbents unless they can be economically processed to assure uniform purity and, therefore, consistent performance. Thus, mineral composition varies in many instances because of the presence of impurities which frequently cannot be removed easily during processing. Some minerals cannot be put into the desired physical form and still maintain sufficient stability. Many minerals, such as naturally occurring zeolites, are not found in extensive deposits in the form of a material of relatively uniform pure composition. Therefore, naturally occurring minerals such as zeolites have very

2

limited application to the purification of large volumes of liquid fuel wastes.

Accordingly, an object of this invention is the provision of a method for adsorbing radio cesium from liquid fuel wastes with a synthetically produced zeolite which may be readily prepared in the desired purity from abundant raw material.

A more particular object of this invention is the provision of an economical method for adsorbing radio cesium from low level liquid radioactive wastes which contain also an appreciable concentration of other ions, especially sodium ion.

Further objects and advantages will be apparent from a description of this invention which follows.

After extensive experimentation with the adsorptive properties of scores of silicates, including various naturally occurring and synthetic silicates, we have discovered that a particular type of synthetic zeolitic silicate, which may be readily prepared from abundant raw material in the desired purity, possesses exceptional adsorptive selectivity for radio cesium ions. Further, we have found that selectivity for radio cesium ions is not a property of zeolites as a class. In fact, this property apparently cannot be predicted merely on the basis of the chemical analysis of a zeolite. Further, we have also discovered that no direct correlation generally exists between base-exchange capacity or surface area of a zeolite solid and its effectiveness as a selective adsorbent for cesium. Thus, for example, a synthetic crystalline silicate of the approximate empirical formula



and having an exceptionally high base-exchange capacity of about 660 meq./100 gm. was found to have a cesium adsorption value (defined hereafter) of only about 21% after 48 hours. This cesium adsorption value did not differ significantly from the cesium adsorption value of another synthetic hydrous sodium aluminosilicate of the same  $Na_2O/Al_2O_3/SiO_2$  mol ratio which had a much lower base-exchange capacity of 183 meq./100 gm. On the other hand, a different sodium aluminosilicate having substantially the same base-exchange capacity as the second-mentioned sodium aluminosilicate was found to be more than four times as effective in adsorbing cesium cations as was either of the aforementioned hydrated sodium aluminosilicates.

Briefly stated, in accordance with this invention, aqueous waste liquids containing radio cesium in solution, such as, for example, liquids obtained by leaching spent uranium nuclear fuel with acid solutions, are directly contacted with particles of a hydrous synthetic amorphous zeolite containing about 4 to 14 mols of  $SiO_2$  per mol of  $Na_2O$  and about 1 to 2 mols of  $Al_2O_3$  per mol of  $Na_2O$ , said zeolite having been obtained by precipitating oxides of sodium, aluminum and silicon in intimate association with finely divided particles of pre-precipitated silica. After being contacted with the zeolite in this manner for a time sufficient for the zeolite to adsorb substantially completely all of the radio cesium in the waste liquid, the cesium-depleted waste liquid may be discharged to waste or, in some instances, it may be further processed for removal of other radioactive elements before disposal. The zeolite with sorbed radio cesium can be sealed in a suitable container which is then buried in a suitable geological formation.

This process appears to be especially applicable to the purification of low level waste liquids, especially substantially neutral waste liquid containing an excess of sodium ions over radio cesium ions, since these liquids do not lend themselves to disposal procedures which are feasible with waste liquids having a higher concentration of radioactive elements.

More specifically, the synthetic zeolites used in carrying out this invention are those sodium aluminosilicates prepared by the precipitation process described in U.S. Patent No. 2,848,346 to Bertorelli, to which reference is made herein. As described in the Bertorelli patent, the production of these unique zeolites involves the following essential steps: (1) forming a suspension of fine free precipitated silica in a dilute aqueous solution of a salt of aluminum and a mineral acid; (2) forming a dilute aqueous solution of sodium silicate having a mol ratio of  $\text{SiO}_2$  to  $\text{Na}_2\text{O}$  of about 1 to about 3.6; and (3) combining these two liquid compositions with agitation while keeping the reaction medium alkaline so as to precipitate the desired zeolite which is then separated from the reaction medium, dried and sometimes pulverized.

Step (1), viz., the formation of a suspension of precipitated silica in dilute aqueous solution of aluminum salt, is conveniently carried out by decomposing kaolin clay (a mineral of the empirical formula



with sulfuric acid. This results in the formation of aluminum sulfate and a silica residue of the starting clay. Many methods for decomposing kaolin clay or calcined kaolin clay with acid are known and methods other than those described in the above-mentioned patent to Bertorelli can be used. Kaolin clay of sufficient purity is in extremely abundant supply as compared with naturally occurring zeolites such as clinoptilolite and erionite and, therefore, the supply of the ultimate zeolite which can be produced from kaolin clay is very great as compared with the supply of available naturally occurring zeolites.

The mol ratio of  $\text{SiO}_2$  to  $\text{Na}_2\text{O}$  in the composition is varied by changing the quantity of alkali metal silicate solution (2) mixed with suspension (1).

Using kaolin clay which has been substantially completely decomposed by acid into an aluminum salt of a mineral acid and a silica residue, the mol ratio of  $\text{Al}_2\text{O}_3$  to  $\text{Na}_2\text{O}$  in the zeolite product will be about 1:1. The mol ratio of  $\text{Al}_2\text{O}_3$  to  $\text{Na}_2\text{O}$  in the product can be increased by using concentrated sulfuric acid as the mineral acid and calcining the sulfuric acid reacted clay intermediate product so as to decompose partially the aluminum sulfate constituent of the reaction product producing alumina and volatile oxides of sulfur which are withdrawn from the system. The nonvolatile residue obtained by calcination of the acid reacted kaolin clay, consisting of a mixture of aluminum sulfate, alumina and silica residue of kaolin clay is slurried in water in the usual manner. The slurry is mixed as described above with sodium silicate, using the sodium silicate in amount sufficient to react only with the aluminum sulfate in the slurry.

Synthetic amorphous zeolites useful in carrying out our adsorptive contact process may contain from 4 to 14 mols of  $\text{SiO}_2$  per mol of  $\text{Na}_2\text{O}$ . Zeolites having from 8 to 12 mols of  $\text{SiO}_2$  per mol of  $\text{Na}_2\text{O}$  have been found to have exceptional adsorptive selectivity for radiocesium.

The type of zeolites obtained by the general procedure described above is amorphous to X-rays, in distinct contrast to natural silicate minerals previously recommended for use as cesium adsorbents which are crystalline. The base-exchange capacities of the amorphous zeolites which are used in carrying out the adsorption process of this invention vary somewhat with composition, especially with the  $\text{SiO}_2/\text{Al}_2\text{O}_3$  ratio of the zeolite and are typically within the range of about 180 to 230 meq./100 gm. The surface area values of the zeolites lie within a relatively broad range, also depending on composition, and may be as low as about 60  $\text{m}^2/\text{gm}$ . to as high as about 260  $\text{m}^2/\text{gm}$ .

Our adsorptive contact process can be carried out at ambient temperature. Contact of the waste liquid containing radiocesium with the adsorbent zeolite can be for a time within the range of about  $\frac{1}{2}$  hour to 96 hours. Total pickup of radiocesium with our zeolite is rapid as compared with pickup of prior art radiocesium adsorbents

and, generally speaking, contact periods of more than about 12 hours may not effect a significant improvement in radiocesium adsorption. The zeolite may be in the form of the precipitated powder or the powder may be pelleted by means known to those skilled in the art to form granular particles of the desired form and shape.

Following are examples which are illustrative of the practice and utility of this invention.

Synthetic amorphous zeolites within the scope of this invention were tested for cesium adsorption in the presence of interfering ions and compared to several natural materials (clinoptilolite, illite, grundite and erionite) that have shown promise as adsorbents for  $\text{Cs}^{137}$ . The composition of the test waste aqueous solution was made up to simulate an actual low level radioactive waste liquid.

#### PREPARATION OF SYNTHETIC ZEOLITE SAMPLES FROM KAOLIN CLAY

Synthetic amorphous sodium aluminosilicate hydrates of the type used in carrying out the adsorption process of this invention were produced by reaction of sodium silicate with a slurry of precipitated silica in aluminum sulfate solution (obtained by decomposing kaolin clay with concentrated sulfuric acid).

(a) A zeolite of the approximate composition



was prepared as follows:

Georgia kaolin clay was mixed with 190% acid dosage of 93% sulfuric acid and the mixture placed in a vented gas fired oven at a bed temperature of 600° F. for 6 hours. This product had a V.M. of 68.4%, an  $\text{SO}_3$  content of 32.9% and a free acid content of 6.2%, weight basis. (The term "V.M." refers to volatile matter which is the weight percentage of a material eliminated when it is heated to essentially constant weight at about 1800° F. Acid dosage is the weight of 100% acid based on the volatile free weight of the clay, expressed on a percentage basis.)

A slurry of the acid reacted clay was prepared by dispersing 905 gm. of the reacted clay in 1750 gm. of distilled water (160° F.) containing 48 gm.  $\text{NaOH}$  to neutralize the free acid. The slurry was cooled, then diluted with distilled water to make a slurry containing approximately 11% by weight of total aluminum and silicon (expressed as oxides).

A solution of 19.5% by weight of sodium disilicate ( $\text{Na}_2\text{O} \cdot 2\text{SiO}_2$ ) was prepared by diluting type "O" brand sodium silicate solution in an aqueous solution of  $\text{NaOH}$ .

1930 gm. of the sodium disilicate solution was slowly added to 2500 ml. of agitated distilled water until a pH of 10.5-11.0 was obtained. 1005 gm. of the slurry of acid reacted clay was added to the diluted sodium disilicate solution at a rate such that the pH of the resulting slurry was maintained within these limits. After all of the slurry was added, the reaction was allowed to continue for 15 minutes after which the pH of the reaction medium was  $9.0 \pm 0.2$ . The slurry was filtered and the precipitate washed with distilled water until a sulfate free filtrate was obtained. The cake was dried in a forced air oven at 220° F. The product was micropulverized using a 0.020 inch screen.

The product (identified as Sample No. 2) had the following analysis (all oxides are expressed on a volatile free basis):

|                         | Wt. percent |
|-------------------------|-------------|
| $\text{Al}_2\text{O}_3$ | 13.42       |
| $\text{SiO}_2$          | 76.42       |
| $\text{Na}_2\text{O}$   | 8.73        |
| $\text{Fe}_2\text{O}_3$ | 0.23        |
| $\text{TiO}_2$          | 0.62        |
| Total $\text{SO}_3$     | 0.78        |
| F.M. <sup>1</sup>       | 3.43        |
| V.M.                    | 14.25       |

<sup>1</sup> Free moisture, determined by heating the product to essentially constant weight at 220° F.

## (b) A zeolite of the approximate formula



was prepared by the general procedure described above with the exception that the acid reacted kaolin clay had been calcined at 1200° F. for 1½ hours before being slurried with water, thereby eliminating mineral oil which had been used as a reaction medium in forming the mass of acid reacted kaolin clay.

The resulting product (identified hereafter as sample No. 3) had the following analysis (all oxides reported on a volatile free basis):

|                         | Wt. percent |
|-------------------------|-------------|
| $\text{Al}_2\text{O}_3$ | 21.53       |
| $\text{SiO}_2$          | 70.09       |
| $\text{Na}_2\text{O}$   | 6.38        |
| $\text{Fe}_2\text{O}_3$ | 0.25        |
| $\text{TiO}_2$          | 0.64        |
| $\text{SO}_3$           | 0.49        |
| F.M.                    | 4.61        |
| V.M.                    | 13.86       |

## TESTING ADSORBENTS FOR CESIUM ADSORPTION

The method used for testing cesium adsorption was patterned after that used at the Health Physics Division, Oak Ridge National Laboratory, United States Atomic Energy Commission and was as follows:

A stock solution was made up to simulate radioactive waste liquid by incorporating 6.3 mg. of purified  $\text{CsCl}$  in 1 liter of 0.6 N  $\text{NaNO}_3$  (reagent grade). To this stock was added approximately 2.5 microcuries of radiocesium. The radiocesium was in the form of a dilute aqueous solution of the chloride salt containing 45 microcuries of radiocesium in 8 ml. of 1 N  $\text{HCl}$  and was made up by dilution of  $\text{Cs}^{137}\text{Cl}$  in the 1 N  $\text{HCl}$ .

In testing the adsorptive capacity of solid adsorbents for radiocesium adsorption, a 1.6 gram portion of sample of powdered adsorbent was added to 40 ml. of the stock solution in a 50 ml. glass-stoppered volumetric flask. The adsorbent and stock solution were shaken for 30 to 100 minutes and then allowed to stand overnight in the stoppered flask. The next morning a 1 ml. portion of the supernatant solution was withdrawn and was counted three times to determine the  $\text{Cs}^{137}$  content. Each sample was again shaken for approximately one hour and allowed to stand for two days. A 1 ml. portion of superna-

tant was removed from each sample and another count was made.

The plateau for the scaler and Model 163 Scaling Unit was determined with three different standards ( $\text{Cs}^{137}$  rod,  $\text{Cs}^{137}$  disc and U glass) in place in the detector, a DS5-5 Scintillation Detector, a well-type instrument with a T1-activated NaI crystal. The working voltage was found to be 1200 to 1250 volts. The detector was shielded with a lead case especially designed for it. The scaling unit was used at integral counting for the plateau determination, but for the sorption studies differential counting was employed, the discriminator giving a good background of only 8.5 counts per minute.

No detectable adsorption of cesium by the glass-stoppered volumetric flasks was found. The largest error in the results appears to be the standard statistical error due to the magnitude of the counts recorded in the radioactivity determinations.

The results of the cesium adsorption determination and other data on the adsorbent samples are shown in the accompanying table. Surface area measurements were determined by the nitrogen absorption method described by S. Brunauer, P. H. Emmett and E. Teller in their article entitled "Adsorption of Gases in Multi-Molecular Layers," on page 309 of J.A.C.S., vol. 66, April 1944. Base-exchange capacities of the samples were analytically determined by the ammonium acetate exchange method. The composition of reference minerals was checked by standard X-ray powder diffraction procedure.

The adsorption data show that at least about 94% ( $\pm$  about 4%) of the radiocesium was adsorbed after 48 hours' contact by samples No. 1, 2 and 3—representative synthetic amorphous zeolites obtained by precipitating oxides of Na, Si and  $\text{Al}_2\text{O}_3$  in the presence of pre-precipitated silica obtained from acid decomposition of kaolin clay. These samples were at least as effective in a 48 hour contact time as clinoptilolite, sample No. 4, which was the most effective of the minerals reported in the screening test, and were significantly more effective than the illites.

The data also show that adsorption of radiocesium by the synthetic amorphous zeolites, in accordance with this invention, was substantially complete after standing overnight in contrast with most of the naturally occurring minerals, including the crystalline zeolite (sample No. 4), in which case adsorption was improved by more prolonged contact of the adsorbent with the solution.

Cesium adsorption of natural and synthetic silicates  
SYNTHETIC AMORPHOUS ZEOLITES DERIVED FROM KAOLIN CLAY

| Sample No. | Composition of Adsorbent Sample                                                                       | Surface Area, M.²/gm. | Base-Exchange Capacity, Meq./100 gm. | Cesium Adsorption, Percent* |                         |
|------------|-------------------------------------------------------------------------------------------------------|-----------------------|--------------------------------------|-----------------------------|-------------------------|
|            |                                                                                                       |                       |                                      | Sample Standing Overnight   | Sample Standing 48 hrs. |
| 1          | $\text{Na}_2\text{O} \cdot \text{Al}_2\text{O}_3 \cdot 8.0\text{SiO}_2 \cdot 6\text{H}_2\text{O}$ a   | 63                    | 217                                  | 94.9                        | 94.0                    |
| 2          | $\text{Na}_2\text{O} \cdot \text{Al}_2\text{O}_3 \cdot 9.0\text{SiO}_2 \cdot 5\text{H}_2\text{O}$ b   | 263                   | 230                                  | 97.6                        | 97.2                    |
| 3          | $\text{Na}_2\text{O} \cdot 2\text{Al}_2\text{O}_3 \cdot 11.5\text{SiO}_2 \cdot 6\text{H}_2\text{O}$ c | 177                   | 184                                  | (f)                         | 95.9                    |

## NATURALLY OCCURRING MINERALS

|   |                |    |     |      |      |
|---|----------------|----|-----|------|------|
| 4 | Clinoptilolite | 30 | 217 | 83.8 | 93.4 |
| 5 | Illite d       |    |     | 70.5 | 78.9 |
| 6 | Grundite e     |    |     | 70.1 | 68.3 |

a A material supplied under trade name "Zeolex 23" and understood to be made from kaolin clay by process of U.S. Patent No. 2,848,346.

b Preparation described above.

c Preparation described above.

d American Petroleum Institute Research Project, Reference Clay Mineral No. 35.

e A type of illite obtained from Oak Ridge National Laboratory.

f Adsorbent did not settle out to give clear supernatant for testing.

\*All values subject to a rather uniform absolute error of about 4 units in each percentage adsorption value due to magnitude of counts recorded.

We claim:

1. A method for purifying liquid radioactive waste material which comprises contacting an aqueous waste liquid containing radio cesium in solution with a solid synthetic amorphous hydrous zeolite for a time sufficient to adsorb radio cesium in said liquid on particles of said zeolite, and separating waste liquid thus contacted from said zeolite, said zeolite containing 4 to 14 mols of  $\text{SiO}_2$  per mol of  $\text{Na}_2\text{O}$  and from about 1 to 2 mols of  $\text{Al}_2\text{O}_3$  per mol of  $\text{Na}_2\text{O}$  and being obtained by precipitating oxides of sodium, aluminum and silicon in intimate association with finely divided particles of pre-precipitated silica. 10

2. The method of claim 1 in which the mol ratio of  $\text{SiO}_2$  to  $\text{Na}_2\text{O}$  in said zeolite is from 8 to 12. 15

3. A method for purifying an aqueous waste liquid containing a low level of radio cesium in the form of a dissolved salt of a mineral acid which comprises contacting said liquid with a solid synthetic amorphous hydrous zeolite for a time sufficient to adsorb radio cesium on particles of said zeolite, and separating liquid thus contacted from said zeolite, said zeolite containing 4 to 14 mols of  $\text{SiO}_2$  per mol of  $\text{Na}_2\text{O}$  and from about 1 to 2 mols of  $\text{Al}_2\text{O}_3$  per mol of  $\text{Na}_2\text{O}$  and being obtained by precipitating oxides of sodium, aluminum and silicon in intimate association with finely divided particles of pre-precipitated silica. 20

4. The method of claim 3 in which the mol ratio of  $\text{SiO}_2$  to  $\text{Na}_2\text{O}$  in said zeolite is from 8 to 12. 25

5. A method for purifying a substantially neutral spent aqueous waste liquid containing a low level of radio cesium in the form of a nitrate salt and also containing in solution a salt of a nonradioactive cation which comprises contacting said liquid at ambient temperature with particles of a solid synthetic amorphous hydrous zeolite 30 35

for a time within the range of about  $\frac{1}{2}$  to 48 hours, thereby to selectively adsorb radio cesium on particles of said zeolite, and separating liquid thus contacted from said zeolite, said zeolite containing .4 to 14 mols of  $\text{SiO}_2$  per mol of  $\text{Na}_2\text{O}$  and from about 1 to 2 mols of  $\text{Al}_2\text{O}_3$  per mol of  $\text{Na}_2\text{O}$  and being obtained by precipitating oxides of sodium, aluminum and silicon in intimate association with finely divided particles of pre-precipitated silica.

6. The method of claim 5 in which the mol ratio of  $\text{SiO}_2$  to  $\text{Na}_2\text{O}$  in said zeolite is from 8 to 12. 6

7. The method of claim 5 wherein said waste liquid contains sodium ions in excess of ions of radio cesium. 7

#### References Cited in the file of this patent

##### UNITED STATES PATENTS

|           |            |       |               |
|-----------|------------|-------|---------------|
| 943,535   | Gans       | ----- | Dec. 14, 1909 |
| 2,616,847 | Ginell     | ----- | Nov. 4, 1952  |
| 2,848,346 | Bertorelli | ----- | Aug. 19, 1958 |
| 2,916,437 | Gilbert    | ----- | Dec. 8, 1959  |
| 2,974,108 | Alexander  | ----- | Mar. 7, 1961  |
| 3,017,242 | Ames       | ----- | Jan. 16, 1962 |
| 3,030,181 | Milton     | ----- | Apr. 17, 1962 |

##### OTHER REFERENCES

"Removal of  $\text{Cs}^{137}$  and  $\text{Sr}^{90}$  From Aqueous Solution by Ion Exchange on Vermiculite," Sammon et al., At. Energy Research Estab. (Great Britain) R-3274, 14 pp. (1960), cited in Chem. Abstracts, vol. 54 (1960), 23873i.

"Zeolitic Extraction of Cesium From Aqueous Solutions," Ames, U.S. At. Energy Comm., HW-62607, 25 pp. (1959), cited in Chem. Abstracts, vol. 54 (1960), 24077b.

UNITED STATES PATENT OFFICE  
CERTIFICATE OF CORRECTION

Patent No. 3,167,504

January 26, 1965

Walter L. Haden, Jr., et al.

It is hereby certified that error appears in the above numbered patent requiring correction and that the said Letters Patent should read as corrected below.

In the grant, line 1, and in the heading to the printed specification, line 4, name of first inventor, for "Walter L. Hayden, Jr.", each occurrence, read -- Walter L. Haden, Jr. --.

Signed and sealed this 15th day of June 1965.

(SEAL)

Attest:

ERNEST W. SWIDER  
Attesting Officer

EDWARD J. BRENNER  
Commissioner of Patents